

## 1

2,696,430

## STABILIZERS FOR NITRO-CELLULOSE MIXTURES

John A. Gallagher, Indian Head, Md., and Irving Pincus, State College, Pa., assignors to the United States of America as represented by the Secretary of the Navy

No Drawing. Application May 3, 1950,  
Serial No. 159,872

10 7 Claims. (Cl. 52—5)

(Granted under Title 35, U. S. Code (1952), sec. 266)

This invention relates in general to the stabilization of single and double base cellulose nitrate powders by the addition of a small amount of N-alkyl-nitroaniline, or mixtures of these compounds.

## 2

4-nitroaniline, incorporating them into powders, to lower the melting point, and to improve the plasticizing qualities of these compounds.

Other objects of the invention will appear in and be apparent from the specification.

In the preparation of experimental powders for possible stabilizers, several tests are useful to eliminate all but the most promising for addition to the nitrocellulose. The results of these tests for certain of the compounds screened are tabulated for comparison. Samples used in the 134.5° C. heat test are formed by mechanically extruding 12.6 percent pyrocotton with one-half (1/2) percent stabilizer, using ether and alcohol as a solvent. The product is allowed to stand one day in air and is then placed in a vacuum oven for eight (8) hours at 40° C. A standard 134.5° heat test and a 5 hour test are run on the sample. The nitrogen dioxide absorption and viscosity tests are conventional laboratory procedures for these purposes.

## Screening tests for stabilizers

|                               | NO <sub>2</sub> Absorption at 25° C., Pressure in mm. Mercury |            |        |         |       | Viscosity Change <sup>1</sup> (poises) | Heat Test at 134.5° C. Methyl Violet (min.) | 5 hour Test, hrs. |
|-------------------------------|---------------------------------------------------------------|------------|--------|---------|-------|----------------------------------------|---------------------------------------------|-------------------|
|                               | Initial                                                       | 10 seconds | 1 min. | 10 min. | Final |                                        |                                             |                   |
| Diphenylamine-----            | 72                                                            | 32         | 22     | 20      | 20    | .93                                    | 85                                          | 5                 |
| Ethyl-Centralite-----         | 72                                                            | 63         | 48     | 37      | 34    | 1.05<br>.30<br>.37                     | 88<br>82<br>86                              | 5                 |
| N-Methyl-4-nitro aniline----- | 72                                                            | 0          | 0      | 0       | 0     | .58<br>.60<br>.59                      | 103<br>105<br>96                            | 5                 |
| N-ethyl-4-nitro aniline.      | 72                                                            | 7          | 1      | 0       | 0     | .60                                    | 96                                          | 5                 |

<sup>1</sup> Viscosity change at 25° C. for five days using an ethyl Cellosolve solution of cellulose nitrate (12.6% N). The control dropped an average of 30 poises for this period.

The present method of stabilizing single base powders is by adding diphenylamine, and in double base powders by adding centralite. A disadvantage of using diphenylamine as a stabilizer is that it reacts with oxygen of the air and also with oxides of nitrogen to form black or dark colored dyes of unproved structures. It further reacts with nitrogen dioxide and nitric acid to form nitrogen monoxide gas. Centralite also reacts with nitrogen dioxide to form nitrogen monoxide. Since it is the function of a stabilizer to remove these undesirable products, these materials are not as effective in removing oxides of nitrogen as the chemicals herein disclosed.

The N-alkyl-nitroanilines which contain an alkyl group such as methyl, ethyl, isopropyl, etc., and contain a nitro group in the three or four positions on the benzene ring, when mixed in a nitro-cellulose powder, either single or double base, lead to a powder possessing superior stability. N-methyl-4-nitroaniline, N-ethyl-4-nitroaniline, N-isopropyl-3-nitroaniline, N-butyl-3-nitroaniline are examples.

An important object of the present invention is the substitution of from one-half to one percent (up to five percent) of N-ethyl-4-nitroaniline or N-methyl-4-nitroaniline or mixtures thereof in place of diphenylamine in single base nitro-cellulose powders and in place of ethyl centralite in double base nitrocellulose powders.

A further object of the invention is to produce a superior powder of improved stability which does not become discolored by oxidation impurities.

A still further object of the invention is to make the aniline nitrogen sufficiently neutral by the nitro group in N-alkyl-4-nitroanilines, so that it would be compatible with nitroesters and still be a strong absorbent of highly oxidized nitrogen atoms, such as nitric acid and nitrogen tetroxide.

Still a further object of the invention is to prepare a eutectic mixture of N-ethyl-4-nitroaniline and N-methyl-

50 The results of the screening tests indicate that the N-alkyl mononitroanilines possess excellent stabilizing properties for single base powder. They efficiently absorb nitrogen dioxide reducing little or none of it. They further do not affect the viscosity of cellulose nitrate solution as much as diphenylamine. In the heat test which shows the time in minutes to decolorize methyl violet paper, they compare favorably with diphenylamine.

55 Double base powders were prepared by dissolving 60 percent cellulose nitrate (13.47% N), 39 percent nitro-glycerine and 1 percent stabilizer in acetone and evaporating off the acetone at room temperature. The products were extended through a micro-press and placed in a vacuum oven for 7 days at 45° C. The comparative results are shown as follows:

|    | Stabilizer                      | 120° C. Heat Test (Average), Minutes | 110° C. Vacuum Stability Test |
|----|---------------------------------|--------------------------------------|-------------------------------|
|    |                                 |                                      |                               |
| 65 | Ethyl Centralite (Control)----- | 65                                   | 8.32                          |
|    | N-Methyl-4-nitroaniline-----    | 90                                   | 8.37                          |
|    | N-Ethyl-4-nitroaniline-----     | 85                                   | 8.45                          |

70 The heat test records the time in minutes to decolorize methyl violet paper. The vacuum test records the cubic centimeters (cc.) of gas evolved per gram sample for thirty hours at standard temperature and pressure.

75 In operation as a stabilizer, it appears that the nitro group in N-alkyl-4-nitroanilines makes the aniline nitrogen sufficiently neutral, so that it is compatible with nitro-esters, and at the same time is a strong absorbent of highly oxidized nitrogen molecules, such as nitric acid, nitrogen tetroxide, and the like.

80 These results indicate that for double base powders, the N-alkyl-mononitroanilines are approximately one

third more effective than ethyl-centralite in the heat test and are about the same in the vacuum tests, and therefore they possess improved stabilizing properties for such powders.

A new stabilizing composition for both single and double base powders is thus presented which apparently has improved and superior characteristics, producing a better result than the ingredients now commonly known and used as stabilizers.

The invention described herein may be manufactured and used by or for the Government of the United States of America for governmental purposes without the payment of any royalties thereon or therefor.

We claim:

1. A stabilizer comprising an N-alkyl-nitroaniline of not more than 5 percent by bulk in combination with one of the group of cellulose nitrate and cellulose nitrate nitroglycerine.

2. The combination of a nitrocellulose powder and N-alkyl-4-nitroaniline constituting a stabilizer therefor.

3. The combination of a nitrocellulose powder and a stabilizer therefor of a material selected from the group consisting of N-ethyl-4-nitroaniline and N-methyl-4-nitroaniline of not more than 5 percent by bulk.

4. The combination of cellulose nitrate nitroglycerine powder and not more than five percent by bulk of N-methyl-4-nitroaniline constituting a stabilizer therefor.

5. A stabilizer for nitrocellulose powders comprising a mixture of N-ethyl-4-nitroaniline and N-methyl-4-nitroaniline of not more than 5 percent by bulk incorporated

10

5

6. The combination of a nitrocellulose powder and not more than 5 percent by bulk of N-alkyl-4-nitroaniline as a stabilizer therefor.

7. The combination of a nitrocellulose powder and not more than 5 percent by bulk of N-alkyl-nitroaniline as a stabilizer therefor.

#### References Cited in the file of this patent

#### UNITED STATES PATENTS

| Number    | Name               | Date          |
|-----------|--------------------|---------------|
| 875,922   | Holmes             | Jan. 7, 1908  |
| 875,923   | Holmes             | Jan. 7, 1908  |
| 1,329,212 | Snelling et al.    | Jan. 27, 1920 |
| 2,261,630 | Regestein          | Nov. 4, 1941  |
| 2,323,948 | Von Brammer et al. | July 13, 1943 |
| 2,378,594 | Swan et al.        | June 19, 1945 |
| 2,381,015 | Von Brammer et al. | Aug. 7, 1945  |
| 2,383,361 | Bass et al.        | Aug. 21, 1945 |

#### FOREIGN PATENTS

| Number | Country       | Date    |
|--------|---------------|---------|
| 12,746 | Great Britain | of 1912 |

#### OTHER REFERENCES

The Chemistry of Powder and Explosives, by T. L. Davis, John Wiley and Sons, 1943, N. Y., vol. II, pp. 269 and 307-312.